

## UNITED STATES PATENT OFFICE.

LESTER KIRSCHBRAUN, OF CHICAGO, ILLINOIS.

## FELTED WATERPROOF COMPOSITION AND PROCESS OF MAKING SAME.

No Drawing. Application filed May 24, 1920, Serial No. 383,893. Renewed November 7, 1925.

This invention relates to improvements in felted waterproof compositions and process of making same, and has among its salient objects to provide a process which is particularly adapted to be carried on in a multi-cylinder paper forming machine in which the sheet is formed of a plurality of relatively thin felted plies; to provide a process in which the multiplicity of plies are adhesively bound together in the formation of the paper so as to produce a substantially unitary structure; to provide a process which permits the use of fibre stock of different character in the different plies and also the use of variable character of bituminous or analogous binders in the different plies; to provide a process in which the percentage or amount of binder in the various plies can be varied or eliminated entirely out of any one or more plies; to provide a process which will permit the use of relatively cheap fibre stocks which cannot ordinarily be saturated with asphalt or the like by heretofore known methods; to provide a process in which any one or more of the plies may have different color than the other, which can be accomplished either in the binder or fibre or both; to provide a process which can be utilized on a standard multi-cylinder paper machine without any substantial modification of such machine; to provide a novel product of the above character.

In my previously filed application, Serial No. 339,690, filed Nov. 21, 1919, issued as patent No. 1,615,303, I have described in detail the method of converting an adhesive binder such as asphalt into non-adhesive condition, as for example, a non-adhesive emulsion. I have also there described the mixing of said emulsion with paper stock, and the sheeting of such mixture on a paper forming machine. I have also there described the manner in which the extremely finely dispersed particles of asphalt are uniformly distributed throughout the fibres and upon application of heat coalesce to produce a substantially continuous asphaltic film surrounding the fibres. In other words, the particles of asphalt are no longer in discrete form but have united with each other to form a continuous saturating medium distributed throughout the sheet.

In this application, as in the one heretofore filed and above referred to, I first make a non-adhesive emulsified matrix of asphalt (or other analogous binder) water and a colloid,

as for example clay, in which the asphalt forms the internal phase. In this emulsion, the particles of asphalt average about four one-hundredths of a millimeter in diameter, or in other words, microscopic dimensions. 60 This dispersion of the asphalt facilitates the formation of the continuous saturating medium which is a characteristic of my product. This emulsion is then mixed with fibre, either in the beater or at the screen. 65

If the process is to be operated on a five cylinder machine, the character of the fibre stock and asphalt (either or both) may be varied for each ply. For example, the center ply may have a low melting point asphalt 70 as Mexican oil steam distilled asphalt of 105° F. melting point and 175 to 200 penetration. This will give a flexible ply. The fibre may be either rag stock or old newspapers. In the next two or intermediate 75 plies, i. e., those next to the center ply, the asphalt may be an oxidized or air blown asphalt made from the petroleum residuum, of mid-continental oil as for example, Illinois crude. This asphalt may have a melting 80 point of 150° F. and a penetration of 100. The fibre may be bagging or sulphate pulp or mixtures thereof. Sawdust also may be added to any of the three inner plies, in order to open up the sheet. 85

The emulsion for the two outer plies may be made of a relatively hard asphalt, for example, asphaltic compound composed of Gilsonite and asphalt residuum brought to a penetration of ten to fifteen and a melting 90 point of 160° to 175° F. up to as high as 250° F. In these plies fibre may be sulphite screenings, cotton linters, rope waste. The fibres may be colored by dyes, as for example, red, yellow or any color. 95

If desired, the pitch may be colored and in such case might be the residue from super-heated steam distillation of wax tailings from petroleum oil suitably colored with an oil soluble dye. Also a compound such as Gil- 100 sonite fluxed with stearine, pitch may be used to which is added a pigment. Either the binder or the fibre or both may be colored.

In any of the plies, the percentages of the asphalt or binder relative to the fibre may 105 be varied. For complete saturation, it normally takes for each ply 55% to 60% by weight of asphalt, 8% to 12% of clay and the remainder fibre. Also in the outer plies the amount of asphalt may be entirely eliminated. 110

It is to be understood that the sheet is formed and dried in the multi-cylinder paper machine by passing over cylindrical driers in the usual way. A sheet formed in this way 5 may be used for a wide variety of purposes.

By the term "bitumen" or "pitch," as used in the claims, I intend to include these waterproofing substances hereinbefore described.

I claim as my invention:

- 10 1. A waterproof felted composition consisting of a plurality of felted plies, the fibre of one ply being of different character than the fibre of another ply and a continuous coalesced bituminous film containing an emulsifying agent extending through each 70 ply said plies having the characteristics of being simultaneously felted together during the forming operation.
- 15 2. A waterproof felted composition consisting of a plurality of felted plies, the fibre of one ply being of different character than the fibre of another ply and a continuous coalesced bituminous film extending through each 75 ply, and clay incorporated with the bitumen.

3. A waterproof felted composition consisting of a plurality of plies, each containing fibre and a continuous coalesced bituminous film, the bituminous medium in one 80 ply being of a different character than the bituminous medium of another ply.

4. A waterproof felted composition consisting of a plurality of felted fibrous plies, and a bituminous coalesced film extending 85 through each ply, the film in one ply having a higher melting point than the film in another ply.

5. A waterproof felted composition consisting of a plurality of felted fibrous plies, 90 and a bituminous coalesced film extending through each ply, the film in one ply having a lower penetration than the film in another ply.

6. A process of making a waterproof 95 felted composition consisting in passing a mixture of fibre and a non-adhesive emulsified matrix containing water, bitumen and colloidal clay over a multi-cylinder paper forming machine, sheeting and drying the stock to coalesce the bitumen and form a continuous waterproofing film, the emulsified matrix for one ply having a bitumen of different character than the emulsified matrix of another ply.

55 7. A process of making a waterproof felted composition consisting in passing a mixture of fibre and a non-adhesive emulsified matrix containing water bitumen and colloidal clay over a multi-cylinder paper forming machine, sheeting and drying the stock to coalesce the bitumen and form a continuous waterproofing film, the fibres of one ply being of different character than the fibres of the other plies.

8. A waterproof felted composition, 100 consisting of a plurality of felted fibrous plies

and a bituminous substance dispersed with an emulsifying agent extending through each ply in the form of coalesced continuous film, said plies having the structure characteristics of simultaneous formation.

9. A waterproof felted composition, 105 consisting of a plurality of felted fibrous plies and a bituminous substance with an emulsifying agent in the form of a continuous coalesced film extending through each ply, 75 the coalesced substance in one ply having a higher melting point than the substance in another ply.

10. A waterproof felted composition consisting of a plurality of felted fibrous plies 80 and a bituminous substance with an emulsifying agent in the form of a continuous coalesced film extending through each ply, the coalesced substance in one ply having a lower penetration than the substance in another 85 ply.

11. A process of making a waterproof multi-ply sheet consisting in forming a plurality of fibrous plies upon a multi-cylinder machine, the stock of a plurality of said plies 90 having mixed therewith a normally adhesive bitumen in non-adhesive emulsified form, removing the water from the sheet and causing the bitumen to coalesce as a continuous film coating the fibres.

95 12. A waterproof sheet comprising a plurality of fibrous plies, several of said plies having coalesced therethrough a continuous fused waterproof pitchy medium, the plied product having the structural characteristics 100 of simultaneous formation.

13. A process of making a waterproof multi-ply sheet comprising forming a plurality of fibrous plies into a sheet, mixing with the stock of a plurality of said plies before the 105 plies are united a normally adhesive bitumen in non-adhesive emulsified form, removing the water from the sheet and causing the bitumen to coalesce.

14. A process of making a waterproof 110 felted composition, comprising forming a plurality of fibrous plies into a sheet, the stock of each ply having mixed therewith a normally adhesive bitumen in non-adhesive emulsified form, removing the water from the sheet 115 and causing the bitumen to coalesce.

15. A multi-ply sheet comprising a plurality of plies of fibrous stock, each ply having coalesced therethrough a fused waterproof substance in the form of a continuous 120 coalesced film enveloping the fibres and derived from an emulsion of said waterproofing substance and an emulsifying agent and possessing the characteristics of having had the waterproofing material incorporated simultaneously with the formation thereof.

16. A multi-ply waterproof sheet comprising a plurality of fibrous plies, several of said plies having coalesced therethrough a continuous fused waterproofing medium, the fibres 125

- and waterproofing medium contained in one of the plies being interlocked and integrated with the adjacent ply whereby to prevent separation thereof.
- 5 17. A multi-ply waterproofed sheet comprising a plurality of fibrous plies, several of said plies having coalesced therethrough a continuous fused waterproofing film and an emulsifying agent, the fibres and waterproofing medium contained in one of the plies being interlocked and integrated with the adjacent ply whereby to prevent separation thereof. 10

LESTER KIRSCHBRAUN.